

## UNITED STATES PATENT OFFICE

2,351,347

## TURBINE OIL

Daniel B. Luten, Jr., Berkeley, Calif., assignor to  
 Shell Development Company, San Francisco,  
 Calif., a corporation of Delaware

No Drawing. Application June 8, 1942,  
 Serial No. 446,291

5 Claims. (Cl. 252—52)

This invention relates to the production of mineral oil compositions having properties which render them especially suitable for use as lubricants for turbines and as dielectrics for electrical equipment such as transformers. It also deals with lubricating oils containing small amounts of an addition agent which renders the oil highly resistant to oxidation and gum or sludge formation. More particularly, it deals with the use of 2,4-dimethyl-6-tertiary octyl phenol for stabilizing turbine oils against oxidation and gum formation.

In the past, it has been recommended to add various anti-oxidants or gum inhibitors to mineral hydrocarbon oils to improve their oxidation stability. Among the suggested active inhibitors are the xylenols and the trialkylated phenols. Of the latter, one having two methyl and one tertiary butyl group in the 2,4, and 6 positions, respectively, is particularly effective.

Now I have discovered that 2,4-dimethyl-6-tertiary octyl phenol possesses outstanding characteristics which distinguish this compound from related tri-alkylated phenols for use in the particular mineral oil blends herein contemplated. These outstanding characteristics are improved oxidation stability and reduced tendency to disperse iron rust in the compounded oil.

Good turbine oils must show their superior qualities in commercial use. In the lubrication of turbines, oil is constantly circulated from a storage system connected with the turbine to various parts to be lubricated and back to storage. The oil is used over a long period of time, during which time it comes in contact with the atmosphere as well as with water. This contact leads to deterioration of the oil in that the conditions of use are conducive to oxidation and oil so oxidized tends to emulsify with the water slowly accumulated in the circulatory system. Moreover, the practically unavoidable presence of water frequently causes rusting, particularly in the governor mechanism. Further, metallic iron and/or copper, which is always used in the construction of turbine oiling systems, has a catalytic effect on oil oxidation. A good turbine oil must therefore be highly resistant to oxidation in the presence of iron and copper, must not tend to disperse metallic oxidation catalysts throughout the oil and must maintain a reasonably high interfacial tension against water during use.

Turbine oils having the above properties can be produced from well refined lubricating oils of the proper viscosity range, which may be about 75-750 Say. Univ. Sec. at 100° F. by adding to

these lubricating oils about .01% to 1% of 2,4-dimethyl-6-tertiary octyl phenol.

The phenols which may be alkylated to form the useful tertiary octyl antioxidant are either (1) pure 2,4-dimethyl phenol, or (2) a narrow boiling liquid phenol fraction having an A. S. T. M. 5% boiling point of 206-211° C., a 50% boiling point of 210-212° C. and a 95% boiling point of 211-216° C. Preferably the 5% boiling point is not lower than 209° C. and the 95% point not above 213° C. Such fraction normally contains about 60% of 2,4-dimethyl phenol, the most important of the remaining phenols being about 25% 2,5-dimethyl phenol.

Alkylation may be carried out by using as alkylating compound tertiary base octylene such as di-isobutylene or so-called hot acid octylenes; or tertiary octyl chloride, or the corresponding alcohol, or di-tertiary octyl ether.

Catalysts or condensing agents useful in alkylating the phenols are the inorganic poly-oxy acids such as sulfuric acid, sulfonic acids, phosphoric acid, P<sub>2</sub>O<sub>5</sub>, etc.; Friedel-Crafts catalysts such as aluminum chloride, zinc chloride, acid zinc sulfate, tin tetrachloride, ferric chloride, boron trichloride, boron fluoride; complex compounds of Friedel-Crafts catalysts such as halides of Al, B, Fe, Sn, Sb and W, with inactive halide salts as NaCl, HgCl<sub>2</sub>, AgCl, etc., or dissolved in organic liquids such as nitrobenzene, acetone, acetophenone, benzoyl chloride, di-ethyl sulfone, ethyl phenyl sulfone, diphenyl sulfone, di-isopropyl sulfate, ethyl benzol sulfonic acid ester, etc.; acidic clays, silica gel, etc., and combinations of the above. Those familiar with the art know the proper catalysts to use with each of the alkylating compounds mentioned above.

If desired, the reaction may be carried out in dilution of inert solvents for the alkyl phenols such as carbon disulfide, nitrobenzene, paraffins free of reactive tertiary atoms, etc.

Temperatures suitable for our process may vary with the catalyst but usually are between about 0° and 100° C. and the quantities of catalysts may vary from very small amounts to those equalling or slightly exceeding the amount of alkyl phenols present.

The following example illustrates one method of preparation of the 2,4-dimethyl-6-tertiary octyl phenol: Starting material was xylene fraction boiling at about 211° C. and containing 82.5% 2,4-dimethyl phenol and 17.5% 2,5-dimethyl phenol, the latter being relatively unreactive under the conditions of this reaction. To the xylene fraction was added tertiary octyl

chloride, ferric chloride and carbon disulfide. The mixture was refluxed for 8 hours. Carbon disulfide was removed under vacuum. The high boiling residue was dissolved in benzene and the solution was washed with water to remove ferric chloride. The benzene was distilled off under vacuum and thereafter a high boiling distillate was taken overhead which was fractionated at atmospheric pressure to distill unreacted 2,5-dimethyl phenol and to recover a product consisting essentially of 2,4-dimethyl-6-tertiary octyl phenol.

The amounts of inhibitor required to stabilize turbine oil varies somewhat with conditions and the secondary additives in the oil. When used alone, 2,4-dimethyl-6-tertiary octyl phenol is useful up to about 2%, although it rarely needs to exceed about .5% and generally may be between .05% to .3%.

2,4-dimethyl-6-tertiary octyl phenol may be used in combination with other secondary additives such as corrosion inhibitors, e. g. alkyl succinic acids, aromatic imino alpha di-carboxylic acids, etc., E. P. compounds, blooming agents, etc.

The value of the 2,4-dimethyl-6-tertiary octyl phenol as a stabilizer for turbine oil is illustrated below:

A well-refined turbine oil of 150 S. S. U. viscosity at 100° F. free from added oxidation inhibitors was divided into three portions. To one portion was added .2% by weight of 2,4-dimethyl-6-tertiary butyl phenol. To another portion was added .2% by weight of 2,4-dimethyl-6-tertiary octyl phenol.

A 300 cc. sample of each of the doped and undoped oils was placed in individual oxidation tubes. To each sample was added 60 cc. of distilled water. A coil of joined iron and copper wires was placed in each tube so as to extend through the water layer and to within 3 cm. of

the top of the oil layer. The oxidation tubes were set up in a water bath to maintain the temperature of the oil at 95° C.  $\pm$  1°. Oxygen was then bubbled through each tube at the rate of 3 liters per hour. The passage of oxygen was maintained until the oil in each tube darkened and its neutralization number had reached a value of 5.

Results were as follows:

| 10 | Inhibitor                            | Oxidation time |
|----|--------------------------------------|----------------|
| 15 | None                                 | Hours 150      |
|    | 2,4-dimethyl-6-tertiary octyl phenol | 1,980          |
|    | 2,4-dimethyl-6-tertiary butyl phenol | 660            |

I claim as my invention:

1. A highly refined mineral lubricating oil containing less than 2% of 2,4-dimethyl-6-tertiary octyl phenol.
2. A mineral oil composition comprising turbine oil normally susceptible to oxidation under conditions encountered in use and a small amount of 2,4-dimethyl-6-tertiary octyl phenol sufficient to retard oxidation.
3. Turbine oil comprising predominantly a refined mineral lubricating oil having a viscosity at 100° F. of 75 to 750 Say. Univ. Seconds, and containing dissolved .05% to 2% of 2,4-dimethyl-6-tertiary octyl phenol.
4. Turbine oil comprising predominantly a refined mineral lubricating oil having a viscosity at 100° F. of 75 to 750 Say. Univ. Seconds, and containing dissolved .05% to 3% of 2,4-dimethyl-6-tertiary octyl phenol.
5. A refined hydrocarbon oil subject to oxidation, containing as an active anti-oxidant 2,4-dimethyl-6-tertiary octyl phenol.

DANIEL B. LUTEN, JR.